# EUROPEAN PATENT SPECIFICATION

(11) **EP 1 784 839 B1**
(45) Date of publication and mention of the grant of the patent: **09.05.2012**
(21) Application number: 05788803.4
(22) Date of filing: 22.08.2005
(51) Int. Cl.: H01B 7/29, H01B 3/44, C08K 3/26

(54) **IMPROVED CROSSLINKED AND FLAME RETARDANT AUTOMOTIVE WIRE**
VERBESSERTES QUERVERBUNDENES UND FLAMMHEMMENDES AUTOKABEL
FIL D"AUTOMOBILE RETICULE IGNIFUGE AMELIORE

(30) Priority: 25.08.2004 US 604341 P
(43) Date of publication of application: 16.05.2007
(73) Proprietor: Dow Global Technologies LLC, Midland, MI 48674 (US)
(72) Inventor: COGEN, Jeffrey, M., Flemington, NJ 08822 (US); LIN, Thomas, S., Whippany, NJ 07981 (US); KLIER, John, Midland, MI 48642 (US); WHALEY, Paul, D., Hillsborough, NJ 08844 (US)
(74) Representative: Hayes, Adrian Chetwynd
(86) International application number: PCT/US2005/029901
(87) International publication number: WO 2006/026256

(56) References cited:
- EP-A- 0 393 813
- EP-A- 0 393 959
- EP-A- 1 000 981
- WO-A-2004/074361
- GB-A- 2 262 287
- US-A- 4 543 281

## Description

This invention relates to automotive wire-and-cable applications. In particular, the present invention relates to insulation materials for low-tension primary wire applications.

Generally, automotive wires are required to achieve certain flame retardant performance as set forth by the Society of Automotive Engineers (SAE), industry organizations, or various automobile manufacturers. For example, low tension primary cables must comply with one or more of the specifications of SAE J-1128, ISO-6722, LV 112, Chrysler MS-8288, and Renault 36-36-05-009/-L.

Notably, polyolefin-based formulations, incorporating a metal hydroxide or combinations of metal hydroxides as flame retardants, were designed to fulfil the various specifications. Unfortunately, these solutions have proved inadequate because high amounts of metal hydroxides are required to impart flame retardancy, thereby adding significant cost to formulations.

Within the class of metal hydroxides, certain metal hydroxides raise processing problems. For example, aluminum trihydroxide (ATH) raises compounding rate problems. Specifically, ATH decomposes at temperatures above 175 degrees Celsius. Also, polyolefin-based formulations with halogenated flame retardants pose their own set of problems. Notably, they pose environmental concerns and are expensive solutions.

Accordingly, there is a need for a low-cost alternative to formulations containing high amounts of metal hydroxides or halogenated flame retardants which achieves SAE J-1128 performance and other specifications. More specifically, there is a need for a low-cost, processable alternative which utilized the flame retardant advantages of the metal hydroxides and minimizes the amount of metal hydroxide required to manifest those advantages. There is also a need for a method for selecting such compositions.

The present invention is an automotive wire comprising:
a. a metal conductor;
b. a flame retardant insulation layer, surrounding the metal conductor, prepared from a flame retardant composition comprising
   (i) a crosslinkable thermoplastic polymer,
   (ii) a flame retardant consisting essentially of a metal carbonate being present in an amount greater than or equal to 10 weight percent;
   (iii) a crosslinking agent; and
c. a wire jacket surrounding the insulation layer; and wherein the wire is substantially free of a silicone polymer

The automotive wire passes the specifications of one or more several automotive cable testing protocols: (a) SAE J-1128, (b) ISO-6722, (c) LV 112, (d) Chrysler MS-8288, and (e) Renault 36-36-05-009/-L. The flame retardant composition for making the insulation layer demonstrates economic and processing improvements over conventional solutions. The present invention is also a method for preparing a low tension primary automotive wire and the automotive wire made therefrom.

The present invention provides a method for preparing a low tension primary automotive wire comprising the steps of:
a. selecting a flame retardant composition comprising
   (i) a crosslinkable thermoplastic polymer,
   (ii) a flame retardant consisting essentially of a metal carbonate being present in an amount greater than or equal to 10 weight percent (iii)a crosslinking agent being substantially free
      of a silicone polymer;
b. applying an insulating coating of the flame retardant composition over a metal conductor to form an insulated conductor; and
c. applying a wire jacket over the insulated conductor.

The metal conductor may be any of the well-known metallic conductors used in automotive wire applications, such as copper.

The flame retardant insulation layer is prepared from a flame retardant composition comprising a crosslinkable thermoplastic polymer and a metal carbonate. The metal carbonate is present in an amount sufficient to impart a time to peak heat release (TTPHRR), measured using cone calorimetry with a heat flux of 35 kW/m², of greater than or equal to 140 seconds to a test specimen, having a length and width of 100 mm and a thickness of 1.3 mm. More preferably, the TTPHRR is greater than or equal to 145 seconds. The flame retardant composition is substantially free of a silicone polymer.

The crosslinkable thermoplastic resin is preferably a polyolefin. Suitable polyolefins include ethylene polymers, propylene polymers, and blends thereof. Preferably, the polyolefin polymers are substantially halogen-free.

Ethylene polymer, as that term is used herein, is a homopolymer of ethylene or a copolymer of ethylene and a minor proportion of one or more alpha-olefins having 3 to 12 carbon atoms, and preferably 4 to 8 carbon atoms, and, optionally, a diene, or a mixture or blend of such homopolymers and copolymers. The mixture can be a mechanical blend or an in situ blend. Examples of the alpha-olefins are propylene, 1-butene, 1-hexene, 4-methyl-1-pentene, and 1-octene. The polyethylene can also be a copolymer of ethylene and an unsaturated ester such as a vinyl ester (for example, vinyl acetate or an acrylic or methacrylic acid ester), a copolymer of ethylene and an unsaturated acid such as acrylic acid, or a copolymer of ethylene and a vinyl silane (for example, vinyltrimethoxysilane and vinyltriethoxy silane).

The polyethylene can be homogeneous or heterogeneous. The homogeneous polyethylenes usually have a polydispersity (Mw/Mn) in the range of 1.5 to 3.5 and an essentially uniform comonomer distribution, and are characterized by a single and relatively low melting point as measured by a differential scanning calorimeter. The heterogeneous polyethylenes usually have a polydispersity (Mw/Mn) greater than 3.5 and lack a uniform comonomer distribution. Mw is defined as weight average molecular weight, and Mn is defined as number average molecular weight.

The polyethylenes can have a density in the range of 0.860 to 0.960 gram per cubic centimeter, and preferably have a density in the range of 0.870 to 0.955 gram per cubic centimeter. They also can have a melt index in the range of 0.1 to 50 grams per 10 minutes. If the polyethylene is a homopolymer, its melt index is preferably in the range of 0.75 to 3 grams per 10 minutes. Melt index is determined under ASTM D-1238, Condition E and measured at 190 degree C and 2160 grams.

Low- or high-pressure processes can produce the polyethylenes. They can be produced in gas phase processes or in liquid phase processes (that is, solution or slurry processes) by conventional techniques. Low-pressure processes are typically run at pressures below 7 MPa (1000 pounds per square inch ("psi")) whereas high-pressure processes are typically run at pressures above 105 MPa (15,000 psi)

Typical catalyst systems for preparing these polyethylenes include magnesium/titanium-based catalyst systems, vanadium-based catalyst systems, chromium-based catalyst systems, metallocene catalyst systems, and other transition metal catalyst systems. Many of these catalyst systems are often referred to as Ziegler-Natta catalyst systems or Phillips catalyst systems. Useful catalyst systems include catalysts using chromium or molybdenum oxides on silica-alumina supports.

Useful polyethylenes include low density homopolymers of ethylene made by high pressure processes (HP-LDPEs), linear low density polyethylenes (LLDPEs), very low density polyethylenes (VLDPEs), ultra low density polyethylenes (ULDPEs), medium density polyethylenes (MDPEs), high density polyethylene (HDPE), and metallocene copolymers.

High-pressure processes are typically free radical initiated polymerizations and conducted in a tubular reactor or a stirred autoclave. In the tubular reactor, the pressure is within the range of 175 to 315 MPa (25,000 to 45,000 psi) and the temperature is in the range of 200 to 350 degree C. In the stirred autoclave, the pressure is in the range of 70 to 210 MPa (10,000 to 30,000 psi) and the temperature is in the range of 175 to 250 degree C.

The preferred polymers are copolymers comprised of ethylene and unsaturated esters or acids, which are well known and can be prepared by conventional high-pressure techniques. The unsaturated esters can be alkyl acrylates, alkyl methacrylates, or vinyl carboxylates. The alkyl groups can have 1 to 8 carbon atoms and preferably have 1 to 4 carbon atoms. The carboxylate groups can have 2 to 8 carbon atoms and preferably have 2 to 5 carbon atoms. The portion of the copolymer attributed to the ester comonomer can be in the range of 5 to 50 percent by weight based on the weight of the copolymer. Examples of the acrylates and methacrylates are ethyl acrylate, methyl acrylate, methyl methacrylate, t-butyl acrylate, n-butyl acrylate, n-butyl methacrylate, and 2-ethylhexyl acrylate. Examples of the vinyl carboxylates are vinyl acetate, vinyl propionate, and vinyl butanoate. Examples of the unsaturated acids include acrylic acids or maleic acids.

The melt index of the ethylene/unsaturated ester copolymers or ethylene/unsaturated acid copolymers can be in the range of 0.5 to 50 grams per 10 minutes, and is preferably in the range of 2 to 25 grams per 10 minutes.

Copolymers of ethylene and vinyl silanes may also be used. Examples of suitable silanes are vinyltrimethoxysilane and vinyltriethoxysilane. Such polymers are typically made using a high-pressure process. Use of such ethylene vinylsilane copolymers is desirable when a moisture crosslinkable composition is desired. Optionally, a moisture crosslinkable composition can be obtained by using a polyethylene grafted with a vinylsilane in the presence of a free radical initiator. When a silane-containing polyethylene is used, it may also be desirable to include a crosslinking catalyst in the formulation (such as dibutyltindilaurate or dodecylbenzenesulfonic acid) or another Lewis or Bronsted acid or base catalyst.

The VLDPE or ULDPE can be a copolymer of ethylene and one or more alpha-olefins having 3 to 12 carbon atoms and preferably 3 to 8 carbon atoms. The density of the VLDPE or ULDPE can be in the range of 0.870 to 0.915 gram per cubic centimeter. The melt index of the VLDPE or ULDPE can be in the range of 0.1 to 20 grams per 10 minutes and is preferably in the range of 0.3 to 5 grams per 10 minutes. The portion of the VLDPE or ULDPE attributed to the comonomer(s), other than ethylene, can be in the range of 1 to 49 percent by weight based on the weight of the copolymer and is preferably in the range of 15 to 40 percent by weight.

A third comonomer can be included, for example, another alpha-olefin or a diene such as ethylidene norbornene, butadiene, 1,4-hexadiene, or a ulcyclopentadiene. Ethylene/propylene copolymers are generally referred to as EPRs and ethylene/propylene/diene terpolymers are generally referred to as an EPDM. The third comonomer can be present in an amount of 1 to 15 percent by weight based on the weight of the copolymer and is preferably present in an amount of 1 to 10 percent by weight. It is preferred that the copolymer contains two or three comonomers inclusive of ethylene.

The LLDPE can include VLDPE, ULDPE, and MDPE, which are also linear, but, generally, has a density in the range of 0.916 to 0.925 gram per cubic centimeter. It can be a copolymer of ethylene and one or more alpha-olefins having 3 to 12 carbon atoms, and preferably 3 to 8 carbon atoms. The melt index can be in the range of 1 to 20 grams per 10 minutes, and is preferably in the range of 3 to 8 grams per 10 minutes.

Any polypropylene may be used in these compositions. Examples include homopolymers of propylene, copolymers of propylene and other olefins, and terpolymers of propylene, ethylene, and dienes (for example, norbomadiene and decadiene). Additionally, the polypropylenes may be dispersed or blended with other polymers such as EPR or EPDM. Examples of polypropylenes are described in POLYPROPYLENE HANDBOOK: POLYMERIZATION, CHARACTERIZATION, PROPERTIES, PROFESSING, APPLICATIONS 3-14, 113-176 (E. Moore, Jr. ed., 1996).

Suitable polypropylenes may be components of TPEs, TPOs and TPVs. Those polypropylene-containing TPEs, TPOs, and TPVs can be used in this application.

Examples of suitable metal carbonates include calcium carbonate, calcium magnesium carbonate, and magnesium carbonate. Naturally-occurring metal carbonates are also useful in the present invention, including huntite, magnesite, and dolomite. The metal carbonate is present in an amount greater than or equal to 10 weight percent. Preferably, the metal carbonate is present in an amount greater than or equal to 20 weight percent.

The surface of the metal carbonates may be coated with one or more materials, including silanes, titanates, zirconates, carboxylic acids, and maleic anhydride-grafted polymers. Suitable coatings include those disclosed in U.S. Patent No. 6,500,882. The average particle size may range from less than 0.1 micrometers to 50 micrometers. In some cases, it may be desirable to use a metal carbonate having a nano-scale particle size. The metal hydroxide may be naturally occurring or synthetic.

The flame retardant composition may contain other flame-retardant additives. Suitable non-halogenated flame retardant additives include red phosphorus, silica, alumina, titanium oxides, carbon nanotubes, talc, clay, organo-modified clay, , zinc borate, antimony trioxide, wollastonite, mica, hindered amine stabilizers, ammonium octamolybdate, melamine octamolybdate, frits, hollow glass microspheres, intumescent compounds, and expandable graphite. Suitable halogenated additives include decabromodiphenyl oxide, decabromodiphenyl ethane, ethylene-bis (tetrabromophthalimide), and dechlorane plus.

In addition, the flame retardant composition may contain a nanoclay. Preferably, the nano-clay having at least one dimension in the 0.9 to 200 nanometer-size range, more preferably at least one dimension in the 0.9 to 150 nanometers, even more preferably 0.9 to 100 nanometers, and most preferably 0.9 to 30 nanometers.

Preferably, the nanoclays are layered, including nanoclays such as montmorillonite, magadiite, fluorinated synthetic mica, saponite, fluorhectorite, laponite, sepiolite, attapulgite, hectorite, beidellite, vermiculite, kaolinite, nontronite, volkonskoite, stevensite, pyrosite, sauconite, and kenyaite. The layered nanoclays may be naturally occurring or synthetic.

Some of the cations (for example, sodium ions) of the nanoclay can be exchanged with an organic cation, by treating the nanoclay with an organic cation-containing compound. Alternatively, the cation can include or be replaced with a hydrogen ion (proton). Preferred exchange cations are imidazolium, phosphonium, ammonium, alkyl ammonium, and polyalkyl ammonium. An example of a suitable ammonium compound is dimethyl, di(hydrogenated tallow) ammonium. Preferably, the cationic coating will be present in 15 to 50% by weight, based on the total weight of layered nanoclay plus cationic coating. In the most preferred nanoclay, the cationic coating will be present at greater than 30% by weight, based on the total weight of layered nanoclay plus cationic coating. Another preferred ammonium coating is octadecyl ammonium.

The composition may contain a coupling agent to improve the compatibility between the crosslinkable thermoplastic polymer and the nanoclay. Examples of coupling agents include silanes, titanates, zirconates, and various polymers grafted with maleic anhydride. Other coupling technology would be readily apparent to persons of ordinary skill in the art and is considered within the scope of this invention.

In addition, the flame retardant composition may contain other additives such as antioxidants, stabilizers, blowing agents, carbon black, pigments, processing aids, peroxides, cure boosters, scorch inhibitors, and surface active agents to treat fillers may be present.

The wire jacket is made of a flexible polymer material and is preferably formed by melt extrusion.

In an alternate embodiment, the present invention is a method for preparing a crosslinked, low tension primary automotive wire. The steps of the invented method comprise (a) selecting a flame retardant composition for an insulating layer, (b) applying the selected flame retardant composition as an insulating layer over a metal conductor to form an insulated conductor, and (c) crosslinking the insulating layer, and applying a wire jacket over the insulated conductor. Suitable crosslinking methods include peroxide, e-beam, moisture cure, and other well known methods.

In a preferred embodiment, the present invention is a low tension primary automotive wire prepared from the previously-described method. Additionally, it is believed that the flame retardant composition of the present invention is useful in appliance applications.

### EXAMPLES

The following examples illustrate the invention.

For each of the following exemplified compositions, the insulating compositions were compounded using a laboratory-scale Brabender mixer and analyzed using limiting oxygen index (LOI) and cone calorimetry. The LOI was conducted according to ASTM D-2863 on a 127mm x 6.4mm x 3.2mm test specimen. The cone calorimetry was conducted according to ASTM E-1354 on a 100mm x 100mm x 1.3mm test specimen with a heat flux of 35 kW/m2 without grids. The cone calorimetry measurements include peak heat release rate (PHRR) in kW/m², time to peak heat release rate (TTPHRR) in seconds, time to ignition (TTI) in seconds, fire growth rate index (FIGRA) in kW/m²s, and fire performance index (FPI) in s-m²/ kW. The FIGRA is calculated by dividing the PHRR by the TTPHRR. The FPI is calculated by dividing the TTI by the PHRR.

The following materials were used for the exemplified compositions. The ethylene-ethyl acrylate (EEA) had a melt index of 1.30g/10 minutes, a density of 0.93g/cc, and an ethyl acrylate comonomer content of 15 weight percent. The EEA was obtained from The Dow Chemical Company. It is commercially available as Amplify™ EA 100. The ethylene-vinyl acetate (EVA) had a melt index of 2.50g/10 minutes, a density of 0.94g/cc, and a vinyl acetate comonomer content of 18 weight percent. The EVA was obtained from DuPont. It is commercially available as Elvax™ 460. The ethylene/octene copolymer had a melt index of 4.0g/10 minutes and a density of 0.9 g/cc. The ethylene/octane copolymer was obtained from The Dow Chemical Company. It is commercially available as Attane™ 4404.

The calcium carbonate (CaCO3) was ground and coated with a fatty acid and had an average particle size of 3.5 µm (microns). The nanoclay was a synthetic organo-magadiite prepared as described in Patent Cooperation Treaty Application Serial No. WO 01/83370.

The zinc stearate was obtained as a standard polymer grade. The zinc oxide had a surface area of 9m²/g and was obtained as Kadox™ 911P from Zinc Corporation of America. Irganox 1010 tetrakis [methylene (3,5-di-tert-butyl-4-hydroxyhydro-cinnamate)] methane is available from Ciba Specialty Chemicals Inc.

The compositions were extruded onto 18-gauge/19-strand wires and subjected to 10 MRad of 4.5 MeV electron beam to crosslink the insulating compositions.

### Nonconforming Example 1

**TABLE I**

| **Components** | **N. Ex. 1** |
|---|---|
| EEA | 64.90 |
| EVA | |
| ATH | |
| CaCO3 | 30.00 |
| Mg(OH)2 | |
| Nanoclay | 5.00 |
| Zinc stearate | |
| Zinc oxide | |
| Irganox 1010 | 0.10 |
| Silicone concentrate | |
| **Wire Extrusion Parameters** | |
| RPM | 50 |
| PSI | 2000 |

For the following data, the SAE J-1128 average burn time must be less than 70 seconds for the composition to pass. The MS-8288 average burn time must be less than 30 seconds for the composition to pass.

**TABLE II**

| **Properties** | **N. Ex. 1** |
|---|---|
| Density | 1.19 |
| LOI | 22 |
| PHRR | 308.5 |
| TTPHRR | 97.5 |
| TTI | 54 |
| FIGRA | 3.2 |
| FPI | 0.18 |
| **SAE J-1128 Burn Test** | |
| Burned to clamp? | yes |
| Overage Burn Time (seconds) | 132 |
| Pass | no |
| **MS-8288 Burn Test** | |
| Burned to clamp? | no |
| Average Burn Time (seconds) | 74 |
| Pass | no |

The cone calorimetry results were correlated to passing SAE J-1128 and MS-8288 formulations. Flame retardant compositions having a TTPHRR greater than or equal to about 140 seconds passed both the SAE J-1128 and MS-8288 tests.

Accordingly, flame retardant compositions, containing a metal carbonate, for the insulation layer of low tension primary automotive wire should be selected based upon having a time to peak heat release rate greater than or equal to about 140 seconds.

### Flame Retardant Compositions: Example 2 and Reference Example - 3

**TABLE III The following formulations for Examples 2 - 3 represent compositions that will pass both the SAE J-1128 and MS-8288 tests.**

| **Components** | **Ex. N 2.** | **Reference Ex. 3** |
|---|---|---|
| EEA | | 49.90 |
| EVA | | |
| Ethylene/Qctene Copolymer | 49.90 | 50.00 |
| CaC03 | 50.00 | |
| Mg(OH)2 | | |
| Silica | | |
| Polydimethylsiloxane | | |
| Irganox 1010 | 0.10 | 0.10 |
| Silicone concentrate | | |
| **Properties** | | |
| Density | 1.35 | 1.40 |
| LOI | 21 | 25 |
| PHRR | 167 | 450 |
| **TTPHRR** | **150** | **148** |
| TTI | 80 | 67 |
| FIGRA | 1.1 | 3.0 |
| FPI | 0.48 | 0.15 |

## Claims

1. An automotive wire comprising:
a. a metal conductor;
b. a flame retardant insulation layer, surrounding the metal conductor, prepared from a flame retardant composition comprising
(i) a crosslinkable thermoplastic polymer,
(ii) a flame retardant consisting essentially of a metal carbonate being present in amount sufficient to impart a time to peak heat release (TTPHRR), measured using cone calorimetry with a heat flux of 35 kW/m², of greater than or equal to about 140 seconds to a test specimen,
having a length and width of 101.6 mm and a thickness of 1.3 mm, the amount being greater than or equal to 10 weight percent and
(iii) a crosslinking agent;
c. a wire jacket surrounding the insulation layer; and wherein the wire is substantially free of a silicone polymer.

2. The automotive wire of Claim 1 wherein the crosslinkable thermoplastic resin being a polyolefin.

3. The automotive wire of Claim 1 wherein the metal carbonate being selected from the group consisting of calcium carbonate, calcium magnesium carbonate, and magnesium carbonate.

4. The automotive wire of Claim 1 wherein the metal carbonate being present in amount greater than or equal to about 20 weight percent.

5. A method for preparing a low tension primary automotive wire comprising the steps of:
a. selecting a flame retardant composition comprising
(i) a crosslinkable thermoplastic polymer,
(ii) a flame retardant consisting essentially of a metal carbonate being present in amount sufficient to impart a time to peak heat release (TTPHRR), measured using cone calorimetry with a heat flux of 35 kW/m², of greater than or equal to about 140 seconds to a test specimen, having a length and width of 101.6 mm and a thickness of 1.3 mm being present in an amount greater than or equal to 10 weigth percent and
(iii) a crosslinking agent being substantially free of a silicone polymer;
b. applying an insulating coating of the flame retardant composition over a metal conductor to form an insulated conductor; and
c. applying a wire jacket over the insulated conductor.

6. A low tension primary automotive wire prepared according to Claim 5.

## Patentansprüche

1. Autokabel, umfassend:
a. einen metallischen Leiter;
b. eine flammhemmende Isolierschicht, die den metallischen Leiter umgibt und aus einer flammhemmenden Zusammensetzung hergestellt ist, die Folgendes umfasst:
(i) ein vernetzbares thermoplastisches Polymer,
(ii) einen Flammhemmer, der im Wesentlichen aus einem Metallcarbonat besteht, das in ausreichender Menge vorhanden ist, um eine Zeit bis zur maximalen Wärmefreisetzung ("Time to Peak Heat Release" = TTPHRR), gemessen mittels Kegelkalorimetrie mit einer Wärmestromdichte von 35 kW/m², an ein Prüfstück mit einer Länge und Breite von 101,6 mm und einer Dicke von 1,3 mm von größer oder gleich etwa 140 Sekunden zu verleihen, wobei die Menge größer oder gleich 10 Gew.-% beträgt, und
(iii) ein Vernetzungsmittel;
c. einen Kabelmantel, der die Isolierschicht umgibt; und wobei das Kabel im Wesentlichen frei ist von einem Siliconpolymer.

2. Autokabel nach Anspruch 1, wobei das vernetzbare thermoplastische Harz ein Polyolefin ist.

3. Autokabel nach Anspruch 1, wobei das Metallcarbonat aus der aus Calciumcarbonat, Calciummagnesiumcarbonat und Magnesiumcarbonat bestehenden Gruppe ausgewählt ist.

4. Autokabel nach Anspruch 1, wobei das Metallcarbonat in einer Menge von größer oder gleich etwa 20 Gew.-% vorliegt.

5. Verfahren zur Herstellung eines spannungsarmen primären Autokabels, mit den folgenden Schritten:
a. Auswählen einer flammhemmenden Zusammensetzung, die Folgendes umfasst:
(i) ein vernetzbares thermoplastisches Polymer,
(ii) einen Flammhemmer, der im Wesentlichen aus einem Metallcarbonat besteht, das in ausreichender Menge vorhanden ist, um eine Zeit bis zur maximalen Wärmefreisetzung ("Time to Peak Heat Release" = TTPHRR), gemessen mittels Kegelkalorimetrie mit einer Wärmestromdichte von 35 kW/m², an ein Prüfstück mit einer Länge und Breite von 101,6 mm und einer Dicke von 1,3 mm von größer oder gleich etwa 140 Sekunden zu verleihen, wobei die Menge größer oder gleich 10 Gew.-% beträgt, und
(iii) ein Vernetzungsmittel, das im Wesentlichen frei ist von einem Siliconpolymer;
b. Aufbringen einer Isolationsbeschichtung aus der flammhemmenden Zusammensetzung über einem metallischen Leiter, um einen isolierten Leiter zu bilden; und
c. Aufbringen eines Kabelmantels über dem isolierten Leiter.

6. Spannungsarmes primäres Autokabel, das nach Anspruch 5 hergestellt ist.

## Revendications

1. Fil pour automobiles comprenant :
a. un conducteur métallique ;
b. une couche isolante ininflammable, entourant le conducteur métallique, préparée à partir d'une composition ininflammable comprenant :
(i) un polymère thermoplastique réticulable,
(ii) un ignifuge constitué essentiellement d'un carbonate métallique présent en une quantité suffisante pour donner un délai de dégagement de chaleur maximal (TTPHRR), mesuré en utilisant un calorimètre à cône avec un flux de chaleur de 35 kW/m² supérieur ou égal à environ 140 secondes, à une éprouvette ayant une longueur et une largeur de 101,6 mm et une épaisseur de 1,3 mm, la quantité étant supérieure ou égale à 10 pour cent en poids, et
(iii) un agent de réticulation ;
c. une gaine entourant la couche isolante ;
et dans lequel le fil est substantiellement exempt de polymère silicone.

2. Fil pour automobiles selon la revendication 1, dans lequel la résine thermoplastique réticulable est une polyoléfine.

3. Fil pour automobiles selon la revendication 1, dans lequel le carbonate métallique est choisi dans l'ensemble comprenant le carbonate de calcium, le carbonate de calcium et de magnésium et le carbonate de magnésium.

4. Fil pour automobiles selon la revendication 1, dans lequel le carbonate métallique est présent en une quantité supérieure ou égale à environ 20 pour cent en poids.

5. Procédé de préparation d'un fil primaire à basse tension pour automobiles comprenant les étapes suivantes :
a. sélection d'une composition ininflammable comprenant :
(i) un polymère thermoplastique réticulable,
(ii) un ignifuge constitué essentiellement d'un carbonate métallique présent en une quantité suffisante pour donner un délai de dégagement de chaleur maximal (TTPHRR), mesuré en utilisant un calorimètre à cône avec un flux de chaleur de 35 kW/m² supérieur ou égal à environ 140 secondes, à une éprouvette ayant une longueur et une largeur de 101,6 mm et une épaisseur de 1,3 mm, et qui est présent en une quantité supérieure ou égale à 10 pour cent en poids, et
(iii) un agent de réticulation substantiellement exempt de polymère silicone ;
b. application d'un revêtement isolant fait de la composition ininflammable sur un conducteur métallique pour former un conducteur isolé ; et
c. application d'une gaine sur le conducteur isolé.

6. Fil primaire à basse tension pour automobiles préparé selon la revendication 5.
